

F. VON WURSTEMBERGER.

PROCESS FOR THE PREVENTION OF SELECTIVE CORROSION OF TUBES AND MACHINERY  
PARTS OF COPPER OR COPPER CONTAINING ALLOYS.

APPLICATION FILED JUNE 7, 1919.

1,335,209.

Patented Mar. 30, 1920.

Fig.1



Fig.2



Inventor  
Franz von Wurstemberger  
By Henry Orth Jr. Atty.

# UNITED STATES PATENT OFFICE.

FRANZ VON WURSTEMBERGER, OF ZURICH, SWITZERLAND, ASSIGNOR TO AKTIEN-  
GESELLSCHAFT DER MASCHINENFABRIKEN ESCHER WYSS & CIE., OF ZURICH,  
SWITZERLAND.

## PROCESS FOR THE PREVENTION OF SELECTIVE CORROSION OF TUBES AND MACHINERY PARTS OF COPPER OR COPPER CONTAINING ALLOYS.

1,335,209.

Specification of Letters Patent. Patented Mar. 30, 1920.

Application filed June 7, 1919. Serial No. 302,627.

*To all whom it may concern:*

Be it known that I, FRANZ VON WURSTEMBERGER, a citizen of the Republic of Switzerland, residing at Hardturmstrasse 19, Zurich, Switzerland, have invented certain new and useful Improvements in Processes for the Prevention of Selective Corrosion of Tubes and Machinery Parts of Copper or Copper Containing Alloys; and I do hereby declare the following to be a clear, full, and exact description of the invention, such as will enable others skilled in the art to which it appertains to make and use the same, reference being had to the accompanying drawing, and to letters or figures of reference marked thereon, which form a part of this specification.

The invention consists of a process for the prevention of selective corrosion of tubes and machinery parts of copper or copper containing alloys which are in contact with water containing ions for instance water containing chlorids and of contrivances used for the employment of the process.

Selective corrosion is understood to be that phenomenon whereby fluids which, according to their chemical composition, will attack one portion of metallic parts immersed therein, or in contact therewith, and not other portions.

This phenomenon, known as "pitting," occurs, for instance, on anodes of copper immersed in sodium salt solutions  $\text{Na}_2\text{CO}_3$ , under the influence of electrolysis, or on aluminium anodes in chlorid solutions, for instance,  $\text{NaCl}$  or  $\text{MgCl}_2$ . In practice it is known as the cause of destruction of pump impellers and tube sets of copper and copper containing alloys which are in contact with sea water or with water which conducts electricity, owing to the presence of any kind of salt which it contains in solution.

Careful investigations have shown that the cause of selective corrosion is entirely due to the alteration of the surface of the metallic parts in question and not to the metal not being homogeneous, and that the phenomenon is due to electrolytically different qualities which the different areas acquire under the influence of certain deposits. As such slightly soluble salts of the metals in question come into consideration and ac-

cordingly selective corrosion does not occur in liquids which attack the metal and transform it into an easily soluble salt. The production of selective corrosion is due to the presence of different factors of a chemical and physical nature which are dependent on the nature of the metal in question as also on the salts contained in the water.

One quality which water producing selective corrosion must possess at any rate is a certain electric conductivity. It does not follow however that all water conducting electricity produces selective corrosion.

The behavior of copper and copper containing alloys in contact with water which possess a certain electric conductivity owing to the presence of certain chemicals is briefly explained as follows:

Two different areas of a piece of metal immersed in the water are to be considered as two electrodes in short circuit through the metal itself. At first as soon as the piece of metal is immersed a difference of potential usually arises between the two areas, which difference is dependent on the nature of the layer with which the surfaces of the two areas are covered under the action of oxidation in the air before immersion. The layer may only accidentally be absolutely the same on both areas. Under the influence of this difference of potential one area becomes an anode the other a cathode. However this difference of potential disappears quickly as the electric current produced by it, produces salts on the anode area, through which the concentration of metallic ions there is increased.

The galvanic element formed by the two areas is polarized in this way. By such local electrolysis the whole metal surface is brought in a short time to an equal potential which is higher than the potential of a bright, newly immersed piece of the same metal.

A continuous attack on any spot is only possible where constant anodic depolarization takes place. Such depolarization may occur through mechanical erosion of deposited anodic products or through chemical transformation of those products into slightly soluble compounds, under chemical influence which is equivalent to a reduction

of the concentration of metal ions on this spot. The polarizing layer which is found on copper in water containing chlorid consists of protochlorid of copper  $CuCl$  and basic chlorids of various structure 5  $Cu_x(OH)_xCl_x$ .

As depolarizers have been found: Hot water, which transforms  $CuCl$  by hydrolysis into protoxid of copper, further compounds 10 of all sorts having an alkaline reaction, which transform the  $CuCl$  into  $Cu(OH)_x$ , hydrate of protoxid.

The character of the attack due to such a depolarization depends on the nature of the 15 deposit with alkaline reaction, for instance hydroxid of magnesium deposited in solid form will produce a distinctly limited area of attack according to its slight solubility. On the contrary the easily soluble caustic 20 soda solution  $NaOH$  will act as depolarizer as far as it can spread by diffusion.

As polarizers, *i. e.* chemicals favoring 25 equalization of potential or preventing local attack I have found an addition of acid to be essential. Direct addition of acid however is not practicable because of its secondary action of destroying metals.

On the contrary, an addition of easily 30 soluble hydrolytically decomposing salts of acid reaction as chlorid of aluminium  $AlCl_3$ , and protochlorid of iron  $FeCl_2$ , as well as chlorid of iron  $FeCl_3$ , were found to be good.

According to the process in question for 35 the prevention of selective corrosion on machinery parts of copper or copper containing alloys an easily soluble hydrolytically decomposing salt of acid reaction is added to the water. Such a salt might also be produced immediately in the water which is to 40 be made innocuous, as anode product by sending an electric current through the water and using a suitable metallic anode. The cathodic products are to be carried away.

45 A contrivance suitable for the employment of the process consists of two electrodes through which an electric current is made to pass and is so arranged that the cathodic products are carried away.

50 To avoid injurious secondary electrolysis between electrodes and walls the pipings surrounding the electrodes are to be built of electrically nonconducting material, as for instance clay.

55 For the same purpose the electric tensions employed may be kept low at any rate less than double the tension of polarization, which the two electrodes themselves possess.

The drawing shows schematically a device 60 for carrying out my method with ferric chlorid.

Figures 1 and 2 show a device which can be used in an open channel leading water to a surface condensing plant. Fig. 1 shows 65 the longitudinal section through the channel

and the single parts of the device. Fig. 2 shows the cross section on II-II.

The cooling water is supplied to the condenser 1 (the copper or brass cooling pipes of which must be protected from selective 70 corrosion or pitting) by means of a centrifugal pump 2 from an open channel in which the water flows from left to right. The pump must also be protected against corrosion, as its impeller is of bronze. In the 75 open channel 3 a massive iron anode 4 is arranged before the pump 2. The cathode 5, which is made of any conducting material, say of iron, is surrounded by a clay pipe. An electric current is supplied from any 80 source 6 (for instance from a generator) through both electrodes. The clay pipe 7 which rests on the supports 10, is open underneath toward the channel and is provided with a discharge pipe 8, which keeps the 85 water level in the pipe somewhat lower than the water level in the channel, so that the products of electrolysis, such as soda solution  $NaOH$  and other hydroxids as also hydrogen which form at the cathode 5, are continually carried away. Iron protochlorid ( $FeCl_2$ ) forms at the anode 4, and is carried away by the stream of water, as shown by the dotted arrows 9 in Fig. 1. Ferric protochlorid is transformed partly 90 into a basic chlorid by the air in the water and partly into ferric chlorid, and acts as a preventive of corrosion, both on the bronze 95 wheel of the pump 2 as also on the copper cooling tubes in the condenser 1.

100 The anode 4 should be arranged in such a manner that the strongest electrolytic action takes place at the point (13) farthest from the electric wire (12), in order that the cathode may be used up completely. 105 The dotted arrows 14 show the path of the electric current from the anode 4 to the cathode 5. The intensity of the current must vary according to the quantity of injurious salts contained in the water, and will be adjusted to a minimum by suitably choosing the tension and determining the distance between the anode 4 and the cathode 5.

110 Apparatus other than that shown herein 115 forms the subject matter of my application Ser. No. 303,406, filed July 11, 1919.

I claim:—

1. The process for the prevention of selective corrosion of tubes and machinery parts of copper or copper containing alloys, which are in contact with water containing ions, consisting in introducing into the water an easily soluble hydrolytically decomposable acid reacting salt as preventive means. 120

2. The process for the prevention of selective corrosion of tubes and machinery parts of copper or copper containing alloys, which are in contact with water containing ions consisting of introducing into the water by 130

electrolytic action within the water an easily soluble hydrolytically decomposable acid reacting salt.

3. The process for the prevention of selective corrosion of tubes and machinery parts of copper or copper containing alloys, which are in contact with water containing ions, consisting of the electrolytic production in the corrosive water with which the machinery parts are in contact, of an easily soluble hydrolytically decomposable acid reacting salt as anodic product, the cathodic product being carried away.

4. The process for the prevention of selective corrosion of tubes and machinery parts of copper or copper containing alloys, which are in contact with water containing ions, consisting of the employment of ferric chlorid ( $FeCl_3$ ) as preventive means.

5. The process for the prevention of selective corrosion of tubes and machinery parts of copper or copper containing alloys that are in contact with water containing ions, comprising the electrolytic production of a chlorid of iron as anode product in the corrosive water with which the machinery parts come in contact, the cathode product being carried away.

6. The process for the prevention of selective corrosion or pitting of water-contacting machinery parts containing copper or copper containing alloys, which comprises passing an electric current between iron electrodes inserted in the water and removing the cathode products of electrolysis.

In testimony that I claim the foregoing as my invention I have signed my name.

FRANZ VON WURSTEMBERGER.